

# UNITED STATES PATENT OFFICE.

EUGENE McOUAT, OF NEW YORK, N. Y., AND HENRY W. F. LORENZ, OF SPRINGFIELD, OHIO.

## INCANDESCENT FILAMENT AND PROCESS.

No. 869,013.

Specification of Letters Patent.

Patented Oct. 22, 1907.

Application filed December 6, 1905. Serial No. 290,641.

To all whom it may concern:

Be it known that we, EUGENE McOUAT, a citizen of the United States, and a resident of the city of New York, (borough of Manhattan,) in the county and State 5 of New York, and HENRY W. F. LORENZ, a citizen of the United States, and a resident of Springfield, in the county of Clark and State of Ohio, have invented a new and Improved Incandescent Filament and Process, of which the following is a full, clear, and exact description.

This invention relates to the manufacture of filaments or glowers such as used in incandescent electric lamps.

The object of the invention is to produce a filament having high efficiency and a long period of usefulness.

15 The invention consists in the filament and in the process to be described more fully hereinafter and particularly set forth in the claims.

In preparing a filament according to our invention, we select a core such as a carbon filament, and coat the 20 same with a mixture of silicon and metal, or metals.

We prefer to apply this coat by preparing a caramel solution carrying this mixture of silicon and metal, or metals, in mechanical suspension. In this we dip the carbon filaments in such a way as to deposit a coat 25 thereupon; the filaments then are baked so that the coat becomes dry and incorporated with the filament.

This baking preferably takes place in an indifferent gas, and the temperature is raised to a point sufficiently high to bring about a reaction between the silicon and 30 the metal. In this way a silicid coated filament results. However, the silicid may be incorporated with the filament by other processes, such as the collodion process. This general process consists in dissolving cellulose such as cotton, in nitric acid, hydrochloric 35 acid, or zinc chlorid and the plastic solution obtained is then forced through a die, hardened with alcohol, and afterwards carbonized; according to our invention, while the mass is in the plastic state, we mix with it a quantity of silicon and a metal, both in a finely divided 40 state. The amount of silicon and metal added should be about 50 per cent of the plastic mass, but good results may be obtained with a preparation as low as ten per cent. All of the metals that have a high melting point may be used, except those of the platinum group.

45 Metals which we have particularly in mind are thorium, tungsten, uranium, titanium, tantalum, niobium, vanadium, nickel, cobalt, molybdenum, manganese and chromium; all these metals form silicids. The proportion of silicon to metal we find to be, is about 5 per.

50 cent when using titanium uranium, tungsten and molybdenum; and 35 to 40 per cent of silicon when using thorium, tantalum, niobium, vanadium, nickel, cobalt, manganese and chromium. These proportions are given merely by way of illustration as other proportions 55 were found which give almost as good results.

Our silicid filament may be also made by an impregnation process, in which the entire core of the filament is impregnated with the silicid. In this instance we soak a carbonizable thread in a mixture containing silicon and a metal, and afterward carbonize and convert the silicon into a silicid by a high temperature.

Instead of using silicon and a metal in the process described above, which involves the use of a caramel

solution, we may use directly a silicid in that process, in which case we simply make the caramel solution in

60 which a quantity of silicid is mixed, and the silicid is deposited directly upon the carbon cores by dipping them in the mixture. The filaments are afterwards

baked in the usual manner to harden the coat and carbonize the caramel solution with the silicid on the

70 carbon core. Or, the filament of carbon can be flashed in a mixture of a volatile silicon and volatile metal compound, thus depositing silicon and metal simultaneously upon the carbon core. At a high temperature the

silicon and carbon unite to form a silicid coat. The

75 metal is preferably in the form of titanium tetramethide having the formula  $Ti(CH_3)_4$ , molybdenum tetramethide having the formula  $Mo(CH_3)_4$ ; the silicon may be in the form of a tetramethid,  $Si(CH_3)_4$  or in the form

80 of a hydrid  $SiH_4$ .

Having thus described our invention, we claim as new and desire to secure by Letters Patent.

1. The process of making incandescent lamp filaments which consists in incorporating a metal and silicon in the filament and forming a silicid by reaction between the

85 metal and the silicon components.

2. The process of making incandescent lamp filaments which consists in incorporating a metal and silicon in the filament, and heating said filament thereafter to combine the silicon and metal.

90 3. The process of making incandescent filaments which consists in depositing a metal and silicon on the surface of a core and effecting the formation of a silicid by heat.

4. The process of making incandescent filaments which consists in producing a coat on a core, said coat consisting of a carbonizable binder having particles of finely divided metal and silicon in mechanical suspension therein, whereby said metal and silicon adheres to said core, and forming a silicid and carbonizing said binder by heat.

95 5. As a new article of manufacture, an incandescent lamp filament having a carbonized body with a silicid incorporated therewith.

100 6. An incandescent lamp filament having a silicid as a light emitting substance.

105 In testimony whereof we have signed our names to this specification in the presence of two subscribing witnesses.

EUGENE McOUAT.  
(HENRY W. F. LORENZ.

Witnesses as to the signature of Eugene McOUAT:

JNO. M. RITTER.  
F. D. AMMEN.

Witnesses as to the signature of Henry W. F. Lorenz:

J. E. CONKLIN.  
MARIA LORENZ.